

F. ELLERSHAUSEN.

Refining Cast-Steel.

No. 69,417

Patented Oct. 1, 1867.

Fig. 1.



Fig. 2.



Fig. 3.



Witnesses:

S. C. Klemm  
G. A. Ellershausen

Inventor:

Francis Ellershausen  
By Wm. M. Gandy,  
Attorney.

# United States Patent Office.

FRANCIS ELLERSHAUSEN, OF OTTAWA, CANADA.

*Letters Patent No. 69,417, dated October 1, 1867; patented in Canada September 14, 1867.*

## IMPROVEMENT IN THE MANUFACTURE OF CAST STEEL.

The Schedule referred to in these Letters Patent and making part of the same.

TO ALL WHOM IT MAY CONCERN:

Be it known that I, FRANCIS ELLERSHAUSEN, of Ottawa city, in the Dominion of Canada, have invented a new and useful Improvement in the Manufacture of Cast Steel; and I do hereby declare the following to be a full, clear, and exact description of the same, reference being had to the accompanying drawings, forming part of this specification, in which—

Figure 1 represents a horizontal section of furnace at fire-bars on line A B, figs. 2 and 3.

Figure 2 represents a vertical section of furnace on line C D, fig. 1.

Figure 3 represents a vertical section of furnace on line E F, fig. 1.

Similar letters of reference indicate corresponding parts in the several figures.

In the drawings, O represents the external shell of the furnace, and may be constructed in a square form, as shown in fig. 1, of brick or other suitable material. A chimney of suitable height will be carried up from the furnace, and is marked on the drawings as O'. The inner side of the furnace and chimney is lined with fire-brick, E, arranged in the peculiar form shown in the drawings. The inside of this furnace is divided into two distinct furnaces, A and B, one placed over the other, and separated by a hearth-plate, D, of some refractory material. C is a fire-grate placed near the bottom of the lower furnace A for the reception of the fuel. The division hearth-plate D may be made of plumbago, or other refractory material. For the reception of this plate a cheek or recess is made in the wall, and a suitable allowance made for expansion on all sides, or a shelf or shoulder may be made round the wall sufficiently wide to support the hearth-plate D and to permit it to be easily removed by simply lifting it up. The plate will be of a curved form, as shown in figs. 2 and 3, and possess a declivity toward the point of discharge of about half an inch. F is a suitable aperture through the shell of the furnace, placed about two feet above the hearth-plate. By this aperture is introduced the charge, consisting of fuel and ore, into the upper furnace B for the blooming process. G is a blast pipe to the upper furnace, entering the same about ten inches above the hearth-plate. H is the blast pipe of the lower furnace, and enters the same below the grate-bars, as shown in the drawings. J is a channel for introducing the molten cast iron or carbonized compounds of iron into the upper furnace B, and leads from the hearth of an ordinary blast-furnace. It may be made of clay. K is the feeding-opening or door of the lower furnace for the introduction of fuel into the same. L is a discharge-hole for the molten metal, of about one inch in diameter, placed at the lower end of the hearth-plate. M is a hole for the escape of the slag.

With the foregoing brief description of my invention, to which I have given the name of "Ellershausen's Crucible Furnace for Manufacturing Cast Steel direct from the Iron Ore, or from Iron Ore in connection with Wrought Iron," I will now proceed to describe the mode of working the same. The furnace having been arranged in the manner described, the upper furnace B, in connection with the hearth-plate D, forms a retort, which I term a crucible, to be heated in the inside by charcoal or pure charred peat to a sufficient extent for the blooming process, and on the outside on the bottom by the fire of the lower furnace A, which is fed with fuel adapted for giving an intense heat, combustion being maintained in both furnaces by the blast pipes. After both of the furnaces are heated sufficiently I introduce through the channel J such a proportion of molten carbonized iron into the upper furnace as is required to produce a given quantity of cast steel by the union with wrought iron, (for instance, twenty per cent of highly carbonized iron smelted with eighty per cent of molten iron will give cast steel of about one per cent of carbon.) The process of blooming iron from iron ore in the upper furnace is to be commenced, and such a proportion of blooms of iron has to be sunk in the bath of the cast iron as is required to produce a given quantity of cast steel by the union with carbonized iron. Different qualities of cast steel may be produced by varying the proportions of cast to wrought iron. During the operation the lower furnace is to be kept heated to a sufficient degree to maintain the metal in the upper furnace in a state of fusion. After the blooming process is over the metal is drawn off and moulded into ingots as cast steel. Cast steel thus manufactured is as cheap as wrought iron.

The manufacture of cast steel from iron ore in connection with wrought iron is as follows, viz: After the introduction of carbonized iron into the upper furnace, I smelt wrought iron in the same, with the addition of pulverized iron ore in such quantities that the decarbonization of the smelted wrought iron is effected by the addition of the oxide of iron (iron ore) before it sinks into the bath of the previously introduced carbonized

iron. In this manner worn-out rails of railways may be converted into cast steel, which, if desirable, may be again manufactured into steel rails. Cast steel manufactured by my method, as before described, is both superior in quality and produced at a much less cost than by any of the systems heretofore made use of.

I do not confine myself to the precise details herein set forth, as they may be slightly varied with the form and size of the furnaces employed.

Having thus described my invention, what I claim as new, and desire to secure by Letters Patent, is—

1. The furnace above described, consisting of the retort B, hearth-plate D, and lower fire-chamber A, when the parts are constructed, combined, and arranged in the manner above set forth and for the purpose specified.
2. The hearth-plate D, in a furnace containing the retort B and fire-chamber A, substantially as and for the purpose set forth.

3. The process of obtaining cast steel directly from iron ore, or from iron ore in connection with wrought iron, substantially as above described.

IN WITNESS WHEREOF, I have hereunto set my hand and seal this 10th day of January, 1867.

FRANCIS ELLERSHAUSEN.

Witnesses:

JAMES H. GRIDLEY,

NATHAN K. ELLSWORTH.